

No. 794,206.

PATENTED JULY 11, 1905.

R. R. WALKER.  
ROOFING MATERIAL.  
APPLICATION FILED NOV. 22, 1904.

Fig. 1.



C

Fig. 3.



F

Fig. 2.



Inventor  
Robert R. Walker,

Witnesses

J. Mason Vaughan.  
McC. Johnson.

By

Alvado Moore  
Attorney

## UNITED STATES PATENT OFFICE.

ROBERT R. WALKER, OF EAST LIVERPOOL, OHIO, ASSIGNOR TO  
CHARLES E. WALKER, OF EAST LIVERPOOL, OHIO.

## ROOFING MATERIAL.

SPECIFICATION forming part of Letters Patent No. 794,206, dated July 11, 1905.

Application filed November 22, 1904. Serial No. 233,908.

*To all whom it may concern:*

Be it known that I, ROBERT R. WALKER, a citizen of the United States, residing at East Liverpool, in the county of Columbiana and 5 State of Ohio, have invented certain new and useful Improvements in Roofing Material, of which the following is a specification.

My present invention relates to improvements in roofing materials; and the main object is the provision of a flexible roofing which primarily consists of a body material covered or coated with a material impervious to moisture. To attain these objects, I employ a sheet of woven material and combine 10 with the same a filler composition made of ingredients hereinafter set forth and, if so desired, with felting or paper; but I would have it understood that the main object is to provide a woven material saturated or coated 15 with a filling composition.

In the accompanying drawings, Figure 1 is an enlarged detail sectional view of a portion of the roofing embodying my invention. Fig. 2 is a similar view of a modified form, and 20 Fig. 3 is a similar view of another modified form.

Referring to the drawings, my flexible roofing consists, as shown in Fig. 1, of a strip B of woven material, preferably burlap, the 25 same being located centrally and surrounded upon both sides with a coating C of my filler composition, the ingredients of which will hereinafter appear.

In Fig. 2 of the drawings a modified form 30 is shown in which I provide a central strip G of burlap or woven material surrounded or covered on both sides by means of the filler H, the said filler being coated with a layer K of sand.

In Fig. 3 of the drawings, D designates the 35 woven material, E the upper coating of filler, and F the lower strip of paper, the paper and woven material being secured together by means of my improved filler.

It will thus be seen that I provide a roofing 40 in which the central portion or base consists of a woven material, such as burlap, the said burlap or woven material being made impervious to moisture by means of my improved

filler, which at the same time is held in the 50 sheet by the burlap and greatly lengthens the life of the burlap when in use, the said filler protecting the same when in use.

My improved filler consists of elastic baking japan, asphaltum, and rosin. In producing my improved roofing this filler composition is baked on the burlap in a furnace and is mixed about in the following proportions: elastic baking japan, forty per cent.; asphaltum, fifty per cent., and rosin, ten per 55 cent.

It has been my object in producing this improved roofing to provide a roofing which is not easily torn and which when placed upon the roof greatly outlasts any of the well-known forms of roofing-felts, as the burlap prevents the same from being easily torn, while the filler provides a thick coating which will wear a number of years without the necessity of painting the roof, as is now the 70 case.

From the foregoing description, taken in connection with the drawings, it is evident that I provide a flexible roofing of this character which is the embodiment of simplicity, 75 durability, and inexpensiveness, which is therefore thoroughly efficient and practical in use.

What I claim as new, and desire to secure by Letters Patent, is—

1. A flexible roofing material, consisting of a central section of woven fabric saturated and incased by a moisture-proof material consisting of elastic baking japan, asphaltum and 80 rosin.

2. A flexible roofing consisting of a central section of burlap saturated and incased by a moisture-proof material consisting of elastic baking japan, asphaltum and rosin.

3. A flexible roofing consisting of a central 90 section of woven fabric saturated and incased by a moisture-proof material consisting of elastic baking japan forty per cent., asphaltum fifty per cent., and rosin ten per cent.

4. A flexible roofing consisting of a central section of burlap saturated and incased by a moisture-proof material consisting of elastic

80

85

90

95

baking japan forty per cent., asphaltum fifty per cent., and rosin ten per cent.

5. A flexible roofing consisting of a central section of woven fabric which has saturated and baked thereon elastic baking japan, asphaltum and rosin.

6. A flexible roofing consisting of a central section of burlap, which has saturated and

baked thereon elastic baking japan, asphaltum and rosin.

In testimony whereof I affix my signature in presence of two witnesses.

ROBERT R. WALKER.

Witnesses:

ROSS MERCER,  
L. W. CARMAN.